# EUROPEAN PATENT SPECIFICATION

(11) **EP 3 508 591 B1**
(45) Date of publication and mention of the grant of the patent: **21.10.2020**
(21) Application number: 16798544.9
(22) Date of filing: 02.09.2016
(51) Int. Cl.: C22B 9/00, C22B 21/00

(54) **PROCEDURE AND INSTALLATION FOR ELIMINATING IMPURITIES IN A CONTAMINATED MOLTEN METAL**
VERFAHREN UND VORRICHTUNG ZUR ENTFERNUNG VON VERUNREINIGUNGEN AUS GESCHMOLZENEM METALL
PROCÉDÉ ET APPAREIL POUR ÉLIMINIER DES CONTAMINANTS D'UN MÉTAL FONDU

(43) Date of publication of application: 10.07.2019
(73) Proprietor: Fundación Cidaut, 47151 Boecillo (Valencia) (ES)
(72) Inventor: MAROTO SOTO, José Antonio, 47151 Boecillo (Valladolid) (ES); MORIÑIGO SOTELO, Daniel, 47151 Boecillo (Valladolid) (ES); RIVAS SALMÓN, Ana, 47151 Boecillo (Valladolid) (ES); ÁLVAREZ LÓPEZ, Roberto Manuel, 47151 Boecillo (Valladolid) (ES); ARRANZ DE LA FUENTE, Diego, 47151 Boecillo (Valladolid) (ES); ALCALDE DE LA CUESTA, Maria Estibaliz, 47151 Boecillo (Valladolid) (ES); RODRIGUEZ CARRASCAL, Alicia, 47151 Boecillo (Valladolid) (ES)
(74) Representative: Capitán García, Maria Nuria
(86) International application number: PCT/ES2016/070618
(87) International publication number: WO 2018/042061

(56) References cited:
- US-B1- 6 590 200
- DATABASE WPI Week 199619 Thomson Scientific, London, GB; AN 1996-185239 XP002767642, & JP H08 60263 A (ASAI S) 5 March 1996 (1996-03-05)
- DATABASE WPI Week 200274 Thomson Scientific, London, GB; AN 2002-688158 XP002767643, & KR 2002 0036124 A (HANYANG EDUCATIONAL FOUND) 16 May 2002 (2002-05-16)

## Description

### TECHNICAL FIELD OF THE INVENTION

This invention lies within the field of the elimination of impurities in contaminated metals, also known as purification, the most representative example being that of aluminum alloys contaminated with iron.

### BACKGROUND OF THE INVENTION

In the metallurgical industry treatments are performed on secondary materials that allow such material to be re-used in the production process with properties as similar as possible to those of the primary material but at a much lower cost.

In particular, in aluminum alloys, oxides and iron are the greatest contaminants found. These aluminum alloys are very easily contaminated with iron due to direct contact with tools and molds during the entire production process and the presence of oxides is due to the high reactivity of the metal in the presence of oxygen.

There are numerous studies that have focused on attempting to reduce the presence of impurities in molten metals, more specifically there is a large number of studies aimed at trying to reduce the deleterious effect of the presence of iron by precipitation by gravity, centrifugal methods, addition of neutralizing components, rapid setting or supercritical heating 300°C above the melting point. The precipitation and centrifuge separation processes, such as that of Patent with publication number JPH11229055, do not have industrial interest since they are difficult to implement due to their excessively low efficiency and non-continuous processing. Despite the fact that the neutralizing, rapid setting and supercritical heating processes reduce the impact of iron, they do not eliminate the detrimental effects of its presence.

Currently the only real alternative implemented at an industrial level for eliminating iron consists of the dilution with primary aluminum to reduce the content in iron and other contaminants down to values accepted by the standards, with the high financial costs this entails.

Separation using an electromagnetic force, as stated in Leenov's article (Daniel Leenov, Alexander Kolin "Theory of Electromagnetophoresis. I. Magnetohydrodynamic forces experienced by spherical and Symmetrically oriented cylindrical Particles", The journal of Chemical Physics, vol. 22 No. 4, 1954), which theoretically evaluates the effect that an electromagnetic force causes on a spherical particle, is presented as a new method capable of eliminating the presence of these iron-rich impurities or other contaminants and which could be applied with high efficiency, allowing a continuous procedure of industrial interest. Separation by electromagnetic force has for example been already implemented in processes and apparatuses according to documents JP H08 60263 A, KR 2002 0036124 A and US 6 590 200 B1.

There are preliminary studies that have suggested solving the problem described, such as:
- non-continuous processes that focus on using electromagnetic forces by creating a cylindrical force inside the metal and separating the inclusions by the centrifuge effect, sending them to the walls, as is the case of Yamao's document (Fumitaka Yamao, Kensuke Sassa et al., "Separation of Inclusions in Liquid Metal Using Fixed Alternating Magnetic Field", Tetsu-to-Hagane, vol. 83, No 1, 1997);
- use of a high-power magnetic field to remove inclusions such as that explained in the document by Waki (Norihisa Waki, Kensuke Sassa et al., "Magnetic Separation of Inclusions in Molten Metal Using a High Magnetic Field", Tetsu-to-Hagane, vol. 86, No 6, 2000);

Both processes are based on the separation of the impurities already present within the metal due to the effect of fluid dynamic forces and the difference in densities and not on the elimination of harmful components dissolved within the metal and which may not be separated and eliminated simply with the use of fluid dynamic forces or by movement of the metal.

Leenov's document theoretically reflects how electromagnetic forces may actually affect compounds that may be formed with the impurities to be extracted from the metal.

There are electromagnetic systems for metal decanting that exert electromagnetic forces on the conducting metal, most of which use electrodes that must be introduced into the liquid metal in order to pass an electric current through them, which has two great drawbacks: the new contamination of the metal since there is no metal material that withstands the corrosive effect of molten aluminum, and the electrical risk and requirement for industrial-level insulation these devices require in order to implement it in an industrial process without risk of electrocution.

On the other hand, we also know the use of other metal decanting systems, such as linear induction pumps, which avoid contact with the metal and are more versatile with respect to their properties, using alternating current instead of direct current, as with the electrode systems. However, we have not found any evidence of its use to affect the presence of particles inside a conductive metal.

In all the above, we have not encountered any disclosure of a continuous and efficient process that has been implemented at an industrial level.

In the analysis of more industrial references related to the system proposed we have found the patent with publication number WO/2007/018243, which refers to an industrial system for eliminating impurities contained in the metal without resorting to any metallurgic treatment. As with the documents by Yamao and Waki, this system shall never be capable of eliminating the excess above the standard of elements that are dissolved in the metal since when in solution they present no difference regarding conductivity and are therefore not affected by electromagnetic forces.

Moreover, there is also the problem associated with in-situ contamination of the metal, since the process is performed inside a ferromagnetic duct, and all the time the metal is molten within this duct it shall be contaminated by the iron present in the walls of the container and therefore not only it does not solve the problem, but rather it worsens it.

There is thus still a need for purifying metals contaminated with impurities via installations and a continuous process in liquid state without contact with other metal elements.

### DESCRIPTION OF THE INVENTION

### Problems solved by this invention

This invention is capable of eliminating both exogenous impurities, such as oxides previously formed in the molten metal, for example, as well as endogenous impurities that are dissolved in the metal, the latter being those of greater interest and which shall be affected by a first phase of metallurgical treatment. Thanks to this treatment, the impurities to be eliminated shall become new compounds the electrical conductivity of which shall allow the particles to be eliminated to be affected by an electromagnetic field in an entirely different manner from the base metal.

In a second physical or separation treatment phase an electromagnetic force generated by linear induction pumps is applied that produced a relative movement between the particle and the metal containing it, which allows this to be an external treatment, without contact and safe, without requiring the insertion of any metal component in contact with the molten metal, thus preventing possible contamination, such as the degradation of these components.

The metal is always contained within a ceramic channel or duct, never in contact with metallic components, thus preventing contamination from tools during the entire process.

The purifying process is performed continuously and may be adapted to any melting or maintenance furnace of those commonly used in the foundry industry.

### How this is achieved in this invention

The present invention is established and characterized in the independent claims, while the dependent claims describe additional characteristics thereof.

The object of the invention is a purification process and installations for molten metals contaminated with impurities that is industrially viable. The technical problem to be solved is to configure the elements of the installations and to establish the steps of the process in order to achieve said objective.

The invention is based on the capacity of moving a particle with different conductivity from that of the metal containing it, the base metal, with a difference of at least one order of magnitude, referring to the decimal power (10¹), due to the effect of an electromagnetic field. With this measurement of the difference we refer to ten times both lower or greater, or in other words, a difference of more/less ten times (±10, 10<difference=x-y<10; "x" being the conductivity of the particle and "y" that of the base metal).

Therefore, the first step in the process consists in transforming an impurity, the metallurgical or metallurgical treatment step, in the event that such impurity is dissolved within the metal matrix, as an endogenous impurity, into a final particle with a conductivity of at least one order of magnitude of difference with that of the metal, relating to the decimal power, for which an initial element or compound is added to the molten metal. Therefore, we achieve an intermetallic compound or final particle that can be affected by the action of an electromagnetic field. Therefore, the process includes first of all a metallurgical or metallurgical treatment step to be performed in a furnace, in which to melt and mix the metal to be purified with the necessary alloying elements.

And a second physical or separation treatment step, in which the electromagnetic field is produced that acts upon the molten metal and on the particles of different electrical conductivity, wither exogenous or formed in the previous metallurgical step, from the endogenous particles.

One advantage is that the process is of low cost since these are simple steps that use forces that can be produced economically, using linear induction pumps.

Another advantage is that it is compatible with existing furnaces, since the installation produces the electromagnetic field in an inductive manner and from outside the existing furnaces, unlike methods requiring the insertion of electrodes to apply direct current.

Another advantage is that the duct through which the metal flows in this installation is ceramic and external to the furnace, and therefore simple to separate in the case, for example, of an emergency shutdown.

Another advantage is that the metal is constantly contained in ceramic channels or ducts and reservoirs ceramic, and does not therefore become contaminated with elements from the metal containers and tools, as would happen with iron.

Another advantage is that it is a selective process, which can eliminate impurities without affecting the remaining elements in the base metal alloy, if present, since it shall only affect those elements affected by the metallurgical treatment.

Another advantage is that it can be operated continuously and in an automatic manner with the use of commercial components used in automatic installations, such as controls, automatons, etc.

Another advantage is that the impurities, which usually form a kind of scum or sludge, can be eliminated easily from the container mentioned in Claim 10.

Another advantage is that it can be designed based on the flow rate requirements characteristic of each industrial installation in which it is implemented.

Another advantage is it's low maintenance cost, the same as molten metal decanting systems.

### BRIEF DESCRIPTION OF THE DRAWINGS

This specification is supplemented with a set of drawings illustrating the preferred embodiment, which are never intended to limit the invention.
Figure 1 shows a cross section of a section of the second duct with molten metal and a particle on which the existing forces are represented.
Figure 2 shows a diagram with the elements of the installation, showing a first fusion furnace and a second metallurgical treatment furnace. Boxes with dotted lines show the components for the metallurgical treatment step (M) and for the separation treatment step (S). The curved arrow indicates the sense in which the molten metal travels, which is clockwise.
Figure 3 shows a diagram of the installation in which the first fusion furnace and the second metallurgical treatment furnace of Figure 2 are integrated into a third fusion and metallurgical treatment furnace.
Figures 4, 5 and 6 show respectively microscope photographs of different morphologies of the compound AlSi (FeMn) : in a Chinese character, as a star, as a polygon.

### DETAILED DESCRIPTION OF THE PREFERRED EMBODIMENT OF THE INVENTION

An embodiment of the invention based on the figures is provided below.

The purification process disclosed is capable of eliminating endogenous and exogenous impurities from the contaminated metal, provided that the particles have an electrical conductivity that is different in at least one order of magnitude, with regard to the decimal power, to that of the metal that contains them.

For this to occur, the electromagnetic device (3), Figures 2 and 3, generates an electromagnetic field (B) on the metal with the impurities, perpendicular to a current density (J) that is induced upon the same metal lengthwise to the second duct (6) through which it circulates, such that it produces an electromagnetic force (F_{L}), which according to the Lorentz force law should be perpendicular to B and J.

Figure 1 shows the diagram of forces F_{L}=JxB that act upon the molten metal.

The resulting force from all electromagnetic and fluid dynamic forces that act upon a particle contained within the molten metal on which B and J are applied, with a difference in conductivity of at least one order of magnitude with respect to the decimal power and the metal it is contained in, causes a relative movement of that particle with respect to that of the molten metal, in the separation step (S).

The difference in electric conductivity between the molten metal and the particle to be eliminated shall determine the magnitude and sense of this resulting force, which may be in the same sense as that of the electromagnetic force (F_{L}) or contrary to it.

Figure 1 shows in the black circle the particle and the resulting force that acts upon it when the conductivity of the particle is lower than that of the molten metal, in which case it is in an opposite direction to the electromagnetic force (F_{L}) generated on the metal.

In the event that the impurities to be eliminated do not show the necessary difference in electrical conductivity or that they are dissolved in the liquid metal, a metallurgical treatment (M) must be performed, which combines such impurities with other elements, thus transforming them into new compounds with an electrical conductivity different to that of the metal to be purified by at least one order of magnitude in decimal power, whereas the metal is still in a liquid state and at an optimal working temperature.

One option in order to achieve these compounds is to resort to elements between groups 4 and 7 of the periodic table, namely to eliminate iron, which could be manganese or zirconium.

Another important aspect is the shape of the compound to be eliminated, since the resulting force is greater the greater the volume/surface ratio of the impurity. Thus, for example, in the case of eliminating iron, adding manganese produces the compound AlSi(FeMn), which also has three different morphologies: as a Chinese character (Figure 4), a star (Figure 5), or a polygon (Figure 6). It has been proven that the most advantageous configuration is that of the polygon, since it has a greater volume/surface ratio.

Figure 2 shows a diagram of the installation for eliminating impurities in a contaminated metal that includes a first fusion furnace (1) in which said metal can be melted and which is independent from a second furnace (2) for metallurgical treatment (M). An initial element or compound is added to the molten metal that combines with the impurity in order to form an intermetallic compound or final particle with a suitable electrical conductivity. Both furnaces (1, 2) are connected by a first ceramic duct (5).

After the second furnace (2) there is a second ceramic duct (6) through which the molten metal can travel to the electromagnetic device (3).

In said electromagnetic device an electromagnetic field is created by means of linear induction pumps, the field lines of which are crosswise to the movement of the fluid contained in the second duct (6). There is thus a resulting force (R) acting upon the final particle that is capable of moving it, separation step (S). The action of the magnetic field is performed where the molten metal circulates; for the sake of simplicity we indicate the corresponding duct, although it could also be a deposit close to the electromagnetic device (3) or even inside it.

Figure 3 shows the variant in which the first (1) and second (2) furnaces are integrated into a third fusion and metallurgical treatment (M) furnace (9). Obviously, the first connection duct (5) between the first (1) and second (2) furnaces is removed.

Another option, as shown in Figures 2 and 3, which in order to ensure greater flow rates and efficacy of the process, the configuration includes a boost pump (4) to ensure the required flow rate in the event of a very large installation; form the electromagnetic device (3) exits a third duct (7) that connects to such boost pump (4) from which exits a fourth duct (8) to the corresponding furnace (1, 9). Said boost pump (4), although not shown, may be located anywhere in the installation, even inside any of the furnaces (1, 2, 9), since its function is that inherent to any boost pump, of propelling the fluid passing through it.

Optionally, the electromagnetic device (3) comprises a ceramic reservoir, not shown, in which the particles containing impurities are deposited separately from the molten metal.

## Claims

1. A process of eliminating impurities dissolved in a contaminated molten metal, continuously, such impurities being both exogenous to the molten metal and endogenous to it, **characterized in that** an electromagnetic field (B), generated by linear induction pumps, is applied on the contaminated metal that flows through a second ceramic duct (6) and through which a current density (J) is induced in a longitudinal direction to that of the duct, as a result of the electromagnetic force produced in the metal, Lorentz force (F_{L}), and the fluid dynamic forces derived from the movement of the metal, a resulting force (R) acts on the particle that causes a relative movement of said particle with respect to that of the molten metal, when the difference in electrical conductivity between the molten metal and the particle is of at least one order of magnitude with respect to the decimal power, said difference in conductivity is achieved in endogenous impurities by creating an intermetallic compound or final particle by the reaction between the impurity to be eliminated and the addition of an initial element or compound in a metallurgical step (M) prior to the application of the electromagnetic field, the separation phase (S).

2. A process according to Claim 1 in which the initial element or compound that combines with the impurity is one selected from between groups 4 and 7 of the periodic table.

3. A process according to Claim 1 in which the exogenous particles to be eliminated are oxides of the base metal.

4. A process according to Claim 2 in which in order to eliminate iron the initial element is manganese or zirconium.

5. A process according to Claim 4 in which the intermetallic compound AlSi(FeMn) is obtained, the particles of which acquire a morphology of a Chinese character, a star and/or a polygon.

6. Installation for eliminating impurities dissolved in a contaminated metal, comprising a first fusion furnace (1) in which said metal can be melted and a second metallurgic treatment (M) furnace (2) in which an initial element or compound can be added to the metal so that it combines with the impurities to be eliminated in order to form an intermetallic compound or final particle, **characterized in that** after the second furnace (2) there is a second ceramic duct (6) through which the molten metal can travel to an electromagnetic device (3) that can create an electromagnetic field via linear induction pumps, the field lines of which are perpendicular to the longitudinal axis of said second duct (6), so that a resulting force (R) acts upon the final particle that may oppose that caused by the electromagnetic field on the fluid, Lorentz force (F_{L}), and therefore it is carried through said second duct (6) .

7. A installation according to claim 6 wherein both furnaces (1, 2) are connected via a first ceramic duct (5) .

8. A installation according to claim 6 wherein the first and second furnaces (1, 2) are conformed in a single third furnace (9).

9. A installation according to any of the previous claims in which from the electromagnetic device (3) exits a third duct (7) that connects to a boost pump (4) from which exits a fourth duct (8) to the corresponding furnace (1, 9).

10. A installation according to any of the previous claims in which the electromagnetic device (3) comprises a ceramic reservoir in which the particles containing the impurities are gathered separated from the molten metal.

## Patentansprüche

1. Verfahren zum kontinuierlichen Entfernen von Verunreinigungen aus geschmolzenem Metall, wobei diese Verunreinigungen für das geschmolzene Metall sowohl exogen als auch endogen und **dadurch gekennzeichnet sind, dass** ein elektromagnetisches Feld (B), das von linearen Induktionspumpen erzeugt wird, an das geschmolzene Metall angelegt wird, die durch einen zweiten Keramikkanal (6) fließt und durch die eine Stromdichte (J) in Längsrichtung zu der des Kanals induziert wird, wobei infolge der im Metall erzeugten elektromagnetischen Kraft Lorentzkraft (F_{L}) und den fluiddynamischen Kräften, die sich aus der Bewegung des Metalls ergeben, eine resultierende Kraft (R) auf das Teilchen wirkt, was eine Relativbewegung des Teilchens in Bezug auf die des geschmolzenen Metalls bewirkt, wenn der Unterschied in der elektrischen Leitfähigkeit zwischen dem geschmolzenen Metall und dem Teilchen in Bezug auf die Dezimalleistung mindestens einer Größenordnung entspricht, wobei der Unterschied in der Leitfähigkeit bei endogenen Verunreinigungen durch Erzeugen einer intermetallischen Verbindung oder eines Endteilchens durch die Reaktion zwischen der zu entfernenden Verunreinigung und der Zugabe eines Anfangselements oder einer Verbindung in einem metallurgischen Schritt (M) vor dem Anlegen des elektromagnetischen Feldes, der Trennphase (S), erreicht wird.

2. Verfahren nach Anspruch 1, wobei das Ausgangselement oder die Verbindung, das bzw. die sich mit der Verunreinigung verbindet, aus dem Bereich zwischen den Gruppen 4 und 7 des Periodensystems ausgewählt ist.

3. Verfahren nach Anspruch 1, wobei die zu entfernenden exogenen Teilchen Oxide des Grundmetalls sind.

4. Verfahren nach Anspruch 2, wobei das Anfangselement zum Entfernen von Eisen Mangan oder Zirkonium ist.

5. Verfahren nach Anspruch 4, wobei die intermetallische Verbindung AlSi (FeMn) erhalten wird, deren Teilchen eine Morphologie eines chinesischen Schriftzeichens, eines Sterns und/oder eines Polygons erhalten.

6. Einrichtung zum Entfernen von Verunreinigungen aus geschmolzenem Metall, umfassend einen ersten Schmelzofen (1), in dem das Metall geschmolzen werden kann, und einen zweiten Ofen zur metallurgischen Behandlung (M) (2), in dem dem Metall ein Anfangselement oder eine Verbindung zugesetzt werden kann, sodass es sich mit den zu entfernenden Verunreinigungen verbindet, um eine intermetallische Verbindung oder ein Endteilchen zu bilden, **gekennzeichnet dadurch, dass** nach dem zweiten Ofen (2) ein zweiter Keramikkanal (6) vorhanden ist, durch den das geschmolzene Metall zu einer elektromagnetischen Vorrichtung (3) gelangen kann, die über lineare Induktionspumpen, deren Feldlinien senkrecht zur Längsachse des zweiten Kanals (6) stehen, ein elektromagnetisches Feld erzeugen kann, sodass eine resultierende Kraft (R) auf das endgültige Teilchen wirkt, das möglicherweise entgegengesetzt zu der durch das elektromagnetische Feld auf das Fluid wirkenden LorentzKraft (F_{L}) wirkt, und daher wird sie durch den zweiten Kanal (6) geführt.

7. Einrichtung nach Anspruch 6, wobei beide Öfen (1, 2) über einen ersten Keramikkanal (5) verbunden sind.

8. Einrichtung nach Anspruch 6, wobei der erste und der zweite Ofen (1, 2) in einem einzigen dritten Ofen (9) angeordnet sind.

9. Einrichtung nach irgendeinem der vorhergehenden Ansprüche, wobei aus der elektromagnetischen Vorrichtung (3) ein dritter Kanal (7) austritt, der mit einer Druckerhöhungspumpe (4) verbunden ist, aus der ein vierter Kanal (8) zum entsprechenden Ofen (1, 9) austritt.

10. Einrichtung nach irgendeinem der vorhergehenden Ansprüche, wobei die elektromagnetische Vorrichtung (3) ein Keramikreservoir umfasst, in dem die Teilchen, welche die Verunreinigungen enthaltend, getrennt vom geschmolzenen Metall gesammelt werden.

## Revendications

1. Processus d'élimination en continu de contaminants dissous dans un métal fondu, de tels contaminants étant à la fois exogènes au métal fondu et endogènes à celui-ci, **caractérisé en ce qu'**un champ électromagnétique (B), généré par des pompes à induction linéaires, est appliqué sur le métal contaminé qui s'écoule à travers un deuxième conduit en céramique (6) et à travers lequel une densité de courant (J) est induite dans une direction longitudinale à celle du conduit, en raison de la force électromagnétique produite dans le métal, force de Lorentz (F_{L}), et des forces dynamiques fluides dérivées du mouvement du métal, une force résultante (R) agit sur la particule qui provoque un mouvement réciproque de ladite particule par rapport à celui du métal fondu, lorsque la différence de conductivité électrique entre le métal fondu et la particule est d'au moins un ordre de grandeur par rapport à la puissance décimale, ladite différence de conductivité est obtenue dans des contaminants endogènes en créant un composé intermétallique ou une particule finale par la réaction entre le contaminant à éliminer et l'ajout d'un élément ou composé initial dans une étape métallurgique (M) avant l'application du champ électromagnétique, la phase de séparation (S).

2. Processus selon la revendication 1, dans lequel l'élément ou composé initial qui se combine au contaminant est un élément choisi parmi les groupes 4 et 7 du tableau périodique.

3. Processus selon la revendication 1 dans lequel les particules exogènes à éliminer sont des oxydes du métal de base.

4. Processus selon la revendication 2, dans lequel, pour éliminer du fer, l'élément initial est du manganèse ou du zirconium.

5. Processus selon la revendication 4, dans lequel on obtient le composé intermétallique AlSi (FeMn) dont les particules acquièrent une morphologie de caractère chinois, d'étoile et/ou de polygone.

6. Installation pour éliminer des contaminants dissous dans un métal, comprenant un premier four de fusion (1) dans lequel ledit métal peut être fondu et un deuxième four de traitement métallurgique (M) (2) dans lequel un élément ou composé initial peut être ajouté au métal, de sorte qu'il se combine avec les contaminants à éliminer pour former un composé intermétallique ou une particule finale, **caractérisé en ce qu'**après le deuxième four (2), il y a un deuxième conduit en céramique (6) à travers lequel le métal fondu peut se déplacer vers un dispositif électromagnétique (3) pouvant créer un champ électromagnétique via des pompes à induction linéaires, dont les lignes de champ sont perpendiculaires à l'axe longitudinal dudit deuxième conduit (6), de sorte qu'une force résultante (R) agisse sur la particule finale qui peut s'opposer à celle provoquée par le champ électromagnétique sur le fluide, force de Lorentz (F_{L}), et est donc véhiculée à travers ledit deuxième conduit (6).

7. Installation selon la revendication 6 dans laquelle les deux fours (1, 2) sont reliés via un premier conduit en céramique (5).

8. Installation selon la revendication 6 dans laquelle les premier et deuxième fours (1, 2) sont conformés en un troisième four unique (9).

9. Installation selon l'une quelconque des revendications précédentes, dans laquelle, un troisième conduit (7) sort du dispositif électromagnétique (3) et est relié à une pompe de suralimentation (4) d'où sort un quatrième conduit (8) vers le four correspondant (1, 9).

10. Installation selon l'une quelconque des revendications précédentes, dans laquelle le dispositif électromagnétique (3) comprend un réservoir en céramique dans lequel les particules contenant les contaminants sont rassemblées de manière séparée du métal fondu.
